

## 1

**3,592,656**  
**PHOTOGRAPHIC SILVER HALIDE MATERIALS**  
**SUPERSENSITIZED WITH A COMBINATION OF**  
**A TRIAZOLE AND A CYANINE DYE**

Dugald A. Brooks, Rochester, N.Y., assignor to Eastman  
 Kodak Company, Rochester, N.Y.  
 No Drawing. Filed Sept. 3, 1968, Ser. No. 757,147  
 Int. Cl. G03c 1/28

U.S. Cl. 96—126

6 Claims

### ABSTRACT OF THE DISCLOSURE

Photographic silver halide emulsions are supersensitized with the combination of a photographic spectral sensitizing methine dye and a heterocyclic compound selected from a pyrazole, a 5-pyrazolone, a 3-pyrazolone, a 3,5-pyrazolinedione, a triazole, a tetrazole, a xanthine, an imidazole, an imidazolidine and an imidazolinium salt.

This invention relates to novel photographic silver halide emulsions containing a new supersensitizing combination.

It is well known in the photographic art that certain cyanine dyes extend the spectral sensitivity of photographic emulsions. It is further known that a number of such dyes in combination with each other or with certain other compounds markedly alter the sensitivity of photographic emulsions, for example in relative speed, compared with the individual dyes by themselves in such emulsions. While supersensitizing combinations of the above kind have been proposed for various photographic uses, only a relatively few have proven entirely satisfactory for commercial photographic applications. Consequently there is still need in the art for improved supersensitizing combinations comprising methine cyanine dyes.

It is, accordingly an object of this invention to provide a new class of supersensitizing combinations for photographic silver halide emulsions.

Another object of this invention is to provide novel emulsions containing novel supersensitizing combinations, and photographic elements prepared therewith.

Other objects of the invention will be apparent from this disclosure and the appended claims.

I have now made the important discovery that new and improved supersensitizing combinations for light-sensitive photographic silver halide emulsions are produced with (1) a heterocyclic compound selected from a pyrazole, a 5-pyrazolone, a 3-pyrazolone, a 3,5-pyrazolinedione, a triazole, a tetrazole, a xanthine, an imidazole, an imidazolidine and an imidazolinium salt; and, (2) a photographic spectral sensitizing methine dye.

Especially good results are obtained in accordance with this invention when the heterocyclic compound is a 5-pyrazolone; a 1,2,3,4-tetrazole; a 1,2,4-triazole; an imidazole; or, an imidazolinium salt. Some particularly useful heterocyclic compounds have the following formulas:

(I)



(II)



(III)



## 2

(IIIa)



wherein A represents the atoms required to complete an imidazole nucleus, such as imidazole or benzimidazole; R<sub>3</sub> represents a hydrogen atom, an alkyl group of from 1 to 4 carbon atoms, such as methyl, 2-carboxypropyl, butyl, etc., or an aryl group such as phenyl; R<sub>4</sub> represents an aryl group, such as phenyl or 2,4,6-trichlorophenyl; R<sub>5</sub> represents an aryl group such as phenyl, or an amino group such as an arylamino group, e.g., 3,4-dichloroanilino, anilino, 4-methylsulfonamidophenylamino, or an amido group such as 3,5-disulfobenzamido; R<sub>6</sub> represents a hydrogen atom or an arylthio group such as 3-octadecylcarbamylphenylthio; R<sub>7</sub> represents a hydrogen atom or an aryl group such as phenyl; R<sub>8</sub> represents an aryl group such as phenyl, 4-cyanophenyl, 4-methoxyphenyl, 4-carboxyphenyl, naphthyl, a benzoyl group, or pyridyl (3'-pyridyl or 4'-pyridyl); R<sub>9</sub> and R<sub>11</sub> each represents a hydrogen atom, or an aryl group such as phenyl; and, R<sub>10</sub> represents a hydrogen atom or an amino group.

Typical heterocyclic compounds which can be used in this invention include those listed in the following Table 1.

TABLE 1

| Compound No. | Compound                                                                                                                                                                                                                                                                                                                                                                                                                                                                                                                                     |
|--------------|----------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 30           | I..... 3-(3,4-dichloroanilino)-1-phenyl-5-pyrazolone.<br>II..... 3-anilino-2-(2,4,6-trichlorophenyl)-5-pyrazolone.<br>III..... 3-(4-methylsulfonamidophenylamino)-1-(2,4,6-trichlorophenyl)-5-pyrazolone.<br>IV..... 1,3-diphenyl-5-pyrazolone.<br>V..... 3-(3,5-disulfobenzamido)-1-(2,4,6-trichlorophenyl)-5-pyrazolone.                                                                                                                                                                                                                   |
| 35           | VI..... 3-(4-p-toluenesulfoamidoanilino)-1-(2,4,6-trichlorophenyl)-5-pyrazolone.<br>VII..... 3-(3',4'-dichloroanilino)-1-(2',4',6'-trichlorophenyl)-5-pyrazolone.<br>VIII..... bis[5-methyl-2-p-sulfophenyl-3-pyrazolone-(4)]-methine oxonol.<br>IX..... 3-(3,5-dicarbethoxybenzamido)-4-(3-octadecylcarbamylphenylthio)-1-phenyl-5-pyrazolone.                                                                                                                                                                                              |
| 40           | X..... 1,2-diphenyl-3,5-pyrazolinedione.<br>XI..... p-(3,5-diphenyl-2-pyrazolin-1-yl)benzaldehyde.<br>XII..... 3-benzyl-5-phenyl-4-phenylazopyrazole.<br>XIII..... 1,5-diphenyltetrazole.<br>XIV..... 1,8-diphenyl-5-hydroxy-pseudo-tetrazole.                                                                                                                                                                                                                                                                                               |
| 45           | C <sub>6</sub> H <sub>5</sub><br>$\begin{array}{c} \text{HO}-\text{C}=\text{N}-\text{H} \\    \\ \text{N}-\text{C}=\text{N}-\text{C}_6\text{H}_5 \end{array}$                                                                                                                                                                                                                                                                                                                                                                                |
| 50           | XV..... 5-(3',4-dimethoxyphenyl)tetrazole.<br>XVI..... 5-(4'-cyanophenyl)tetrazole-H <sub>2</sub> O.<br>XVII..... 5-(4'-carboxyphenyl)tetrazole-H <sub>2</sub> O.<br>XVIII..... 5-phenyltetrazole.<br>XXI..... 5-benzoyltetrazole.<br>XXII..... 1,4-bis(5-tetrazolyl)benzene.<br>XXIII..... 5-(1-naphthyl)tetrazole.<br>XXIV..... 5-(p-methoxyphenyl)tetrazole.<br>XXV..... 5-(4'-pyridyl)tetrazole.<br>XXVI..... 5-(3'-pyridyl)tetrazole.<br>XXVII..... 4-(N-methyl-p-toluenesulfonamido)-1-(1-phenyl-5-tetrazolyl)oxy-2-methylthiobenzene. |
| 55           | XXVIII..... 3-amino-5-phenyl-1,2,4-triazole.<br>XXIX..... 3,3'-bis(1,5-diphenyl-1,2,4-triazole).<br>XXX..... 1,5-diphenyl-1,2,4-triazole.<br>XXXI..... 4-amino-3,5-di(p-aminophenyl)-1,2,4-triazole.<br>XXXII..... Poly(1,2,4-triazole).<br>XXXIII..... 4-(5-cyanomethyl-1-phenyl-1,2,4-triazol-3-yl)-benzaldehyde-N-chlorophenylhydrazone.<br>XXXIV..... 3,3'-p-phenylenebis(5-cyanomethyl-1-phenyl-1,2,4-triazole).                                                                                                                        |
| 60           | XXXV..... 4-phenylimidazole.<br>XXXVI..... 2-(4,5-diphenyl-2-imidazolyl)phenol.<br>XXXVII..... 1,3-diphenylimidazolidine.<br>XXXVIII..... 1,3-diphenylimidazolinium perchlorate.<br>XXXIX..... 2-(3-pyridyl)benzimidazole.<br>XL..... $\beta$ -(2-mercaptopbenzimidazolyl)propionic acid.<br>XL..... 3-isopentyl-2,6-dithioxanthine.                                                                                                                                                                                                         |
| 65           |                                                                                                                                                                                                                                                                                                                                                                                                                                                                                                                                              |
| 70           | The above classes of heterocyclic compounds are well known and methods for their preparations are described in the various prior art patent references and literature. Some                                                                                                                                                                                                                                                                                                                                                                  |

of the references relating to a number of the specific compounds mentioned in above Table 1 are included herein for illustrative purposes, for example, reference can be had to Chemical Abstracts 22, P3170<sup>5</sup>; 25, P3364<sup>5</sup>; 32, 5831<sup>9</sup>; 41, P1699e; 45, P7603 c; 47, 4335c; 49, 9153e; 51, 138761; 53, 2216c; 53, 4317d; 54, 14234e; 55, 1644e; 55, 2626c; 55, 16520c; 62, P1778a; etc.

The methine dye spectral sensitizers of the invention are represented by the following formulas:



wherein  $e$  and  $n$  represent a positive integer of from 1 to 2;  $d$  and  $m$  each represents a positive integer of from 1 to 3; L represents a methine linkage, e.g.  $=\text{CH}-$ ,



etc.;  $R_1$  and  $R_2$  each represents an alkyl group, including substituted alkyl (preferably a lower alkyl containing from 1 to 4 carbon atoms), e.g., methyl, ethyl, propyl, isopropyl, butyl, hexyl, cyclohexyl, decyl, dodecyl, etc., and substituted alkyl groups (preferably a substituted lower alkyl containing from 1 to 4 carbon atoms), such as a hydroxyalkyl group, e.g.,  $\beta$ -hydroxyethyl,  $\omega$ -hydroxybutyl, etc., an alkoxyalkyl group, e.g.,  $\beta$ -methoxyethyl,  $\omega$ -butoxybutyl, etc., a carboxyalkyl group, e.g.,  $\beta$ -carboxyethyl,  $\omega$ -carboxybutyl, etc.; a sulfoalkyl group, e.g.,  $\beta$ -sulfoethyl,  $\omega$ -sulfobutyl, etc., a sulfatoalkyl group, e.g.,  $\beta$ -sulfatoethyl,  $\omega$ -sulfatobutyl, etc., an acyloxyalkyl group, e.g.,  $\beta$ -acetoxyethyl,  $\gamma$ -acetoxypropyl,  $\omega$ -butyryloxybutyl, etc., an alkoxy carbonylalkyl group, e.g.,  $\beta$ -methoxycarbonylethyl,  $\omega$ -ethoxycarbonylbutyl, etc., or an aralkyl group, e.g., benzyl, phenethyl, etc., or, any aryl group, e.g., phenyl, tolyl, naphthyl, methoxyphenyl, chlorophenyl, etc.;  $X$  represents an acid anion, e.g., chloride, bromide, iodide, thiocyanate, sulfamate, perchlorate, *p*-toluenesulfonate, methylsulfate, etc.;  $R_{12}$  represents a hydrogen atom, an alkyl group of 1-4 carbon atoms, including substituted alkyl, e.g., methyl, ethyl, isopropyl, butyl, dimethylaminopropyl, benzyl, phenethyl, etc. or an aryl group, e.g., phenyl, tolyl, chlorophenyl, methoxyphenyl, naphthyl, etc.;  $D$  represents an atom of oxygen or sulfur; or the non-metallic atoms necessary to complete a diazole ring, e.g.,  $D$  is  $—NR_{13}—$  wherein  $R_{13}$  is an alkyl group of 1 to 4 carbon atoms, e.g., methyl, ethyl, isopropyl, butyl, etc., or an aryl group such as phenyl, tolyl, chlorophenyl, methoxyphenyl, naphthyl, etc.;  $Z$  and  $Z_1$  each represents the non-metallic atoms necessary to complete the same or different 5- to 6-membered heterocyclic nucleus such as used in cyanine dyes which may contain a second hetero atom such as oxygen, sulfur, selenium or nitrogen, such as the following nuclei:

a thiazole nucleus, e.g., thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 5-phenylbenzothiazole, 4-methoxy-

benzothiazole, 5-methoxybenzothiazole, 6-methoxybenzothiazole, 5-iodobenzothiazole, 6 - iodobenzothiazole, 4-ethoxybenzothiazole, 5-ethoxybenzothiazole, tetrahydrobenzothiazole, 5,6 - dimethoxybenzothiazole, 5,6 - dioxy-methylenebenzothiazole, 5-hydroxybenzothiazole, 6 - hydroxybenzothiazole, naphtho[2,1 - d]thiazole, naphtho[1,2-d]thiazole, 5 - methoxynaphtho[2,3, - d]thiazole, 5-ethoxynaphtho[2,3-d]thiazole, 8 - methoxynaphtho[2,3-d]thiazole, 7-methoxynaphtho[2,3-d]thiazole, 4' - methoxythianaphtho-7',6'-4,5-thiazole, etc.;

an oxazole nucleus, e.g., 4 - methylloxazole, 5 - methyl-oxazole, 4-phenyloxazole, 4,5-diphenyloxazole, 4-ethyl-oxazole, 4,5-dimethylloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 4,6 - dimethylbenzoxazole, 5 - methoxybenzoxazole, 5 - ethoxybenzoxazole, 5-chlorobenzoxazole, 6-methoxybenzoxazole, 5-hydroxybenzoxazole, 6-hydroxybenzoxazole, naphtho[2,1-d]oxazole, naphtho[1,2-d]-oxazole, etc.;

a selenazole nucleus, e.g., 4-methylselenazole, 4-phenylselenazole, benzoselenazole, 5-chlorobenzoselenazole, 5-methoxybenzoselenazole, 5-hydroxybenzoselenazole, tetrahydrobenzoselenazole, naphtho[2,1-d]selenazole, naphtho[1,2-d]selenazole, etc.;

a thiazoline nucleus, e.g., thiazoline, 4-methylthiazoline, etc.;

a pyridine nucleus, e.g., 2-pyridine, 5-methyl-2-pyridine, 4-pyridine, 3-methyl-4-pyridine, etc.;

a quinoline nucleus, e.g., 2-quinoline, 3-methyl-2-quinoline, 5-ethyl-2-quinoline, 6-chloro-2-quinoline, 8-chloro-2-quinoline, 6-methoxy-2-quinoline, 8-ethoxy-2-quinoline, 8-hydroxy-2-quinoline, 4-quinoline, 6-methoxy-4-quinoline, 7-methyl-4-quinoline, 8-chloro-4-quinoline, 1-isoquinoline, 3,4-dihydro-1-isoquinoline, 3-isoquinoline, etc.;

a 3,3 - dialkylindolenine nucleus, e.g., 3,3 - dimethyl-indolenine, 3,3,5-trimethylindolenine, etc. and, an imidazole nucleus, e.g., imidazole, 1-alkylimidazole, 1-alkyl-4-phenylimidazole, 1-alkyl-4,5-dimethylimidazole, benzimidazole, 1 - alkylbenzimidazole, 1 - aryl-5,6-dichlorobenzimidazole, 1-alkyl-1H-naphth[1,2-d]imidazole, 1-aryl-3H-naphth[1,2-d]imidazole, 1-alkyl-5-methoxy-1H-naphtha[1,2-d]imidazole, etc.;

and QQ represents the non-metallic atoms necessary to complete a 5- or 6-membered heterocyclic ketomethylene nucleus of the type used in merocyanine dyes typically containing a hetero atom selected from nitrogen, sulfur, selenium, and oxygen, such as

a 2-pyrazolin-5-one nucleus, e.g., 3-methyl-1-phenyl-2-pyrazolin-5-one, 1-phenyl-2-pyrazolin-5-one, 1-(2-benzothiazolyl)3-methyl-2-pyrazolin-5-one, etc.;

an isoxazolone nucleus, e.g., 3-phenyl-5(4H)-isoxazolone, 3-methyl-5(4H)-isoxazolone, etc.;

an oxindole nucleus, e.g., 1-alkyl-2-oxindoles, etc.;

a 2,4,6-triketohexahydopyrimidine nucleus, e.g., barbituric acid or 2-thiobarbituric acid as well as their 1-alkyl (e.g., 1-methyl, 1-ethyl, 1-propyl, 1-heptyl, etc.) or 1,3-dialkyl (e.g., 1,3-dimethyl, 1,3-diethyl, 1,3-dipropyl, 1,3-diisopropyl, 1,3-dicyclohexyl, 1,3-di-( $\beta$ -methoxyethyl), etc. or 1,3-diaryl (e.g., 1,3-diphenyl, 1,3-di-(p-chlorophenyl) 1,3 - di-(p-ethoxycarbonylphenyl), etc.); or 1-aryl (e.g., 1- phenyl, 1-p-chlorophenyl, 1-p-ethoxycarbonylphenyl), etc.) or 1-alkyl-3-aryl (e.g., 1-ethyl-3-phenyl, 1-n-heptyl-3-phenyl, etc.) derivatives;

a rhodanine nucleus (i.e., 2-thio-2,4-thiazolidinedione series), such as rhodanine, 3-alkylrhodanines, e.g., 3-ethylrhodanine, 3 - allylrhodanine, etc., 3 - carboxyalkylrhodanines, e.g., 3-(2-carboxyethyl)rhodanine, 3-(4-carboxybutyl)rhodanine, etc., 3 - sulfoalkylrhodanines, e.g., 3 - (2 - sulfoethyl)rhodanine, 3-(3-sulfopropyl)-rhodanine, 3-(4-sulfobutyl)rhodanine, etc., or 3-aryl-rhodanines, e.g., 3-phenylrhodanine, etc.;

a 2(3H)-imidazo[1,2-a]pyridone nucleus;

a 5,7 - dioxo-6,7-dihydro-5-thiazolo[3,2-a]pyrimidine nu-

- cleus, e.g., 5,7 - dioxo-3-phenyl-6,7-dihydro-5-thiazolo-[3,2-a]pyrimidine, etc.;
- a 2-thio-2,4-oxazolidinedione nucleus (i.e., those of the 2-thio-2,4-(3H,5H)-oxazoledione series) e.g., 3-ethyl-2-thio-2,4 - oxazolidinedione, 3-(2-sulfoethyl)-2-thio-2,4-oxazolidinedione, 3-(4 - sulfobutyl) - 2-thio-2,4-oxazolidinedione, etc.;
- a thianaphthenone nucleus, e.g., 3-(2H)-thianaphthenone, etc.;
- a 2-thio-2,5-thiazolidinedione nucleus (i.e., the 2-thio-2,5-(3H,4H)-thiazoledione series), e.g., 3-ethyl-2-thio-2,5-thiazolidinedione, etc.;
- a 2,4-thiazolidinedione nucleus, e.g., 2,4-thiazolidinedione, 3-ethyl-2,4-thiazolidinedione, 3-phenyl-2,4-thiazolidinedione, 3- $\alpha$ -naphthyl-2,4-thiazolidinedione, etc.;
- a thiazolidinone nucleus, e.g., 4-thiazolidinone, 3-ethyl-4-thiazolidinone, 3-phenyl-4-thiazolidinone, 3- $\alpha$ -naphthyl-4-thiazolidinone, etc.;
- a 2-thiazolin-4-one nucleus, e.g., 2 - ethylmercapto-2-thiazolin-4-one, 2-alkylphenylamino-2-thiazolin-4-one, 2-diphenylamino-2-thiazolin-4-one, etc.;
- a 2-imino-4-oxazolidinone (i.e., pseudohydantoin) nucleus;
- a 2,4-imidazolidinedione (hydantoin) nucleus, e.g., 2,4-imidazolidinedione, 3-ethyl-2,4-imidazolidinedione, 3-phenyl-2,4-imidazolidinedione, 3- $\alpha$ -naphthyl-2,4-imidazolidinedione, 1,3 - diethyl-2,4-imidazolidinedione, 1-ethyl-3-phenyl - 2,4 - imidazolidinedione, 1-ethyl-3- $\alpha$ -naphthyl - 2,4 - imidazolidinedione, 1,3-diphenyl-2,4-imidazolidinedione, etc.;
- a 2-thio-2,4-imidazolidinedione (i.e., 2 - thiohydantoin) nucleus, e.g., 2-thio-2,4-imidazolidinedione, 3-ethyl-2-thio-2,4-imidazolidinedione, 3 - (4-sulfobutyl)-2-thio-2,4 - imidazolidinedione, 3 - (2-carboxyethyl)-2-thio-2,4-imidazolidinedione, 3 - phenyl-2-thio-2,4-imidazolidinedione, 3- $\alpha$ -naphthyl-2-thio-2,4-imidazolidinedione, 1-ethyl-3-phenyl-2-thio-2,4-imidazolidinedione, 1-ethyl-3- $\alpha$ -naphthyl-2-thio-2,4-imidazolidinedione, 1,3-diphenyl-2-thio-2,4-imidazolidinedione, etc.;
- a 2-imidazolin-5-one nucleus, e.g., 2-propylmercapto-2-imidazolin-5-one, etc.

Typical cyanine spectral sensitizing dyes of the invention represented by Formulas IV, V and VI above include those listed in the following table.

TABLE 2

| Dye No. | Compound                                                                                                                                                              |
|---------|-----------------------------------------------------------------------------------------------------------------------------------------------------------------------|
| A       | 2-[(2-benzothiazolylethiodide)methylene]-3- $\beta$ -methoxy-ethyl-5-[1-methyl-2-(1H)-naphtho[1,2-thiazolidinylidene]- $\alpha$ -phenyl-ethylidene]-4-thiazolidinone. |
| B       | 3,3'-diethyloxathiadcarbocyanine iodide.                                                                                                                              |
| C       | 1'-butyl-3-ethyl-4-phenylthia-4'-carbocyanine iodide.                                                                                                                 |
| D       | 3,3'-diethyloxadcarbocyanine iodide.                                                                                                                                  |
| E       | 2-[(2-benzothiazolylethiodide)methylene]-3-ethyl-5-[4-(3-ethyl-2-benzoxazolylidene)-2-butenyldene]-4-thiazolidinone.                                                  |
| F       | 3,3'-diethyl-4,5,4',5'-naphthosulfonadicarbocyanine iodide.                                                                                                           |
| G       | 2-[(2-benzothiazolylethio-p-toluenesulfonate)methylene]-5-[5-chloro-1,3-diethyl-2(3H)-benzimidazolylidene]ethylidene]-3-ethyl-4-thiazolidinone.                       |
| H       | 5-[1-(3-diethyl-2(3H)-benzimidazolylidene)ethylidene]-3-ethyl-2-(4-quinolylethiodide)-4-thiazolidinone.                                                               |
| I       | 3,3'-diethylselenadicarbocyanine iodide.                                                                                                                              |
| J       | 3,3'-dimethyl-4,5,4',5'-naphthothiadcarbocyanine chloride.                                                                                                            |
| K       | 4-[(2-benzothiazolylethiodide)methylene]-2-(3-ethyl-2(3H)-benzothiazolylidene)-methylene]-6-methyl-4H-pyran.                                                          |
| L       | 1,1'-diethyl-2,2'-cyanine iodide.                                                                                                                                     |
| M       | 3,3'-diethyloxacarbocyanine iodide.                                                                                                                                   |
| N       | 1',3-diethylthia-4'-carbocyanine iodide.                                                                                                                              |
| O       | 1',3-diethyl-oxa-4'-carbocyanine iodide.                                                                                                                              |
| P       | 3,3'-di- $\beta$ -hydroxyethylthiadcarbocyanine iodide.                                                                                                               |
| P'      | 3,3'-di- $\beta$ -hydroxyethylthiadcarbocyanine bromide.                                                                                                              |
| Q       | 3,3'-diethyloxatricarbocyanine iodide.                                                                                                                                |
| R       | 3,3'-diethyl-4,5,4',5'-naphthothiadcarbocyanine iodide.                                                                                                               |
| S       | 3,3'-dimethyl-8,12-diphenoxoxyadcarbocyanine iodide.                                                                                                                  |
| T       | 10-cyano-3,3'-diethyloxadcarbocyanine iodide.                                                                                                                         |
| U       | 3,3'-diethyl-4,5,4',5'-tetraphenylthiazolidinocarbocyanine iodide.                                                                                                    |
| V       | Anhydro-1',(1,3-dimethyl-3-sulfobutyl)-3-ethoxy-4'-carbocyanine hydroxide.                                                                                            |
| W       | Anhydro-3-ethyl-5-phenyl-1'- (4-sulfobutyl)thia-4'-carbocyanine hydroxide.                                                                                            |
| X       | 3,3'-diethylthiadcarbocyanine iodide.                                                                                                                                 |
| Y       | 5-[1-(1-ethyl-2(1H)-naphtho[1,2-d]thiazolin-2-ylidene)-1,3-di- $\beta$ -methoxyethyl]-barbituric acid.                                                                |
| Z       | 2[(2-benzothiazolylethoperchlorate)methylene]-3-(3-dimethylaminopropyl)-5-[1-(methylnaphtho[1,2-d]thiazolin-2-ylidene)-1-phenylethylidene]-4-thiazolidinone.          |

The methine dyes of the invention illustrated by those listed in above Table 2 have been previously described in the literature and methods for their preparations are well known. Included among the more pertinent references are the following.

- Zeh et al. U.S. Pat. No. 2,068,047 issued 1/19/37  
 Koslowsky U.S. Pat. No. 2,107,379 issued 2/8/38  
 Mees U.S. Pat No 2,158,883 issued 5/16/39  
 Carroll et al. U.S. Pat. No. 2,177,635 issued 10/3/39  
 Brooker et al. U.S. Pat. No. 2,213,238 issued 9/3/40  
 Brooker U.S. Pat. No. 2,307,916, issued 1/12/43  
 Brooker et al. U.S. Pat. No. 2,313,922, issued 3/16/43  
 Schneider U.S. Pat. No. 2,374,505 issued 4/24/45  
 Falleson et al. U.S. Pat. No. 2,378,917 issued 6/26/45  
 Brooker U.S. Pat. No. 2,454,629 issued 11/23/48  
 Thompson U.S. Pat. No. 2,535,993 issued 12/26/50  
 Carroll et al. U.S. Pat. No. 2,950,196 issued 8/23/60  
 Jones U.S. Pat. No. 2,961,318 issued 11/22/60  
 Tabor et al. U.S. Pat. No. 3,335,010 issued 8/8/67  
 Brooker et al. U.S. Patent Reissue No. 24,292, Reissued 3/19/57  
 British Pat. No. 435,235 accepted 8/28/35

Dye K can be prepared by heating compounds having the following formulas:



in triethylamine and ethanol, to obtain an intermediate of the formula:



The above intermediate is then reacted with a compound of the formula:



50 by heating in pyridine and triethylamine, to obtain dye K.

According to the invention, one or more of the heterocyclic compounds represented by Formulas I, II, III or IIIa above are incorporated with one or more of the cyanine dyes represented by Formulas IV, V and VI above. The invention is particularly directed to gelatinosilver-halide developing-out emulsions. However, the supersensitizing combinations can also be employed in silver halide emulsions in which the carrier of vehicle is a hydrophilic colloid other than gelatin, such as, for example, albumin, agar-agar, gum arabic, alginic acid, etc., or a hydrophilic resin such as polyvinyl alcohol, polyvinyl pyrrolidone, a cellulose ether, a partially hydrolyzed cellulose acetate, acrylamide polymers, etc., which has no deleterious effect upon the light sensitive silver halide. The heterocyclic compounds of Formulas I, II, III and IIIa and the dyes of Formulas IV, V and VI, can be employed in the combinations of the invention in various concentrations depending upon the particular emulsion, concentration of the silver halide, particular results desired, etc. The optimum concentration of an individual sensitizing dye can be determined in a manner well known to those skilled in the art by measuring the sensitivity of a series of test portions of the same emulsion, each portion containing a different concentration of the sensitizing dye. In general, the heterocyclic compounds in my invention

have little or no sensitizing action by themselves alone in the emulsions employed. Ordinarily, the optimum or near optimum concentration of the cyanine dyes herein is of the order 0.01 to 1.2 g. per mole of silver halide in the emulsion, and that of the heterocyclic compound herein is of the order of from about 0.02 to 5.0 g., but generally in the range of about 0.3 to 1.0 g., per mole of silver halide. The preferred combinations range about from 10 to 50% by weight of the cyanine dye and conversely about from 90 to 50% by weight of the heterocyclic compound.

The methods of incorporating sensitizing dyes in silver halide emulsions are well known to those skilled in the art and these known techniques are employed in dispersing the dyes of the invention in the emulsions. In practicing my invention the sensitizing dyes and the heterocyclic compounds can be directly dispersed in the emulsions, or they can first be dissolved in some convenient solvent, such as pyridine, methyl alcohol, acetone, etc. (or mixtures of such solvents), or diluted with water in some instances, and added to the emulsions in the form of these solutions. If desired, the components can be separately dissolved in a given solvent and added separately to the emulsion, or they can be dissolved in the same or different solvent and these solutions mixed together before addition is made to the silver halide emulsions. The dyes and heterocyclic compounds of the invention are dispersed in the finished emulsions in such manner as to be uniformly distributed throughout the emulsions prior to coating on a suitable support, such as paper, glass, cellulose ester film, polyvinyl resin film (e.g., polystyrene film, polyvinyl chloride film, etc.), polyester film, etc. The following procedure has been found quite satisfactory: Stock solutions of the dyes and heterocyclic compounds of Formulas I, II, III and IIIa and the dyes of Formulas IV, V and VI above are prepared by separately dissolving these in appropriate solvents as described above. Then, to the flowable silver halide emulsion, the desired amount of stock solution of one of the dyes is slowly added while stirring the emulsion. Stirring is continued until the dye is thoroughly incorporated in the emulsion. Then, the desired amount of stock solution of one of the heterocyclic compounds is slowly added to the emulsion while stirring. Stirring is continued until the added materials are incorporated in the emulsion. The supersensitized emulsions can then be coated on a suitable support and the coating allowed to dry. In some instances, it may be desirable to heat the supersensitized emulsion for a few minutes before coating onto the suitable support. The details of such coating techniques are well known to those skilled in the art. The foregoing procedure and proportions are to be regarded only as illustrative. Clearly, the invention is directed to any silver halide emulsion containing a supersensitizing combination of the invention, e.g., gelatino-silver chloride, -chlorobromide, -chloroiodide, -chlorobromoiodide, -bromoiodide, etc., emulsions. Fine grain photographic emulsions, such as those described by Sutherns in U.S. patent application Ser. No. 622,034, filed Mar. 10, 1967, can also be supersensitized in accordance with this invention.

The emulsions of this invention can contain the chemical sensitizers, speed increasing compounds, plasticizers, hardeners and coating aids, and the silver halide grains can be dispersed in any of the binders, that are described and referred to by Graham et al. in U.S. Pat. 3,046,129 issued July 24, 1962.

The following examples are included for a further understanding of the invention.

#### EXAMPLES 1 TO 19

These examples illustrate the supersensitization produced with the compounds containing the pyrazole nucleus in combination with various methane dyes of the invention. The testing procedure and the results thereof are set forth in the following description and Table 3.

The specified cyanine dyes and heterocyclic compounds are identifiable from Tables 1 and 2 above.

To different portions of the same batch of melted gelatino-silver bromoiodide emulsion, containing 0.77 mole percent iodide, of the type described by Trivelli and Smith, Phot. Journal, 79, 330 (1939), are added 80 mg. per mole of silver of dye and the heterocyclic compounds in the proportions given in Table 3 hereinafter. In each case, after being digested at about 50° C. for 10 minutes, the emulsion is coated at a coverage of 432 mg. silver per square foot on a cellulose acetate film support. A sample of each coating is exposed on an Eastman IB Sensitometer to light from a tungsten source modulated by a step-wedge and Kodak Wratten No. 16 filter and processed for three minutes in Kodak Developer D-19 which has the following composition:

|    |                                | G.   |
|----|--------------------------------|------|
|    | N-methyl-p-aminophenol sulfate | 2.0  |
| 20 | Hydroquinone                   | 8.0  |
|    | Sodium sulfite (desiccated)    | 90.0 |
|    | Sodium carbonate (monohydrate) | 52.5 |
|    | Potassium bromide              | 5.0  |
|    | Water to make 1.0 liter.       |      |

and then fixed in a conventional sodium thiosulfate fixing bath, washed and dried. Densitometric measurements are then made of the developed images of each coating. The relative speed values are determined by the exposure necessary to produce a density of 0.3 above fog, an arbitrary relative speed of 100 being chosen for the control containing only dye. The results are listed in the following table together with the values for gamma and fog.

TABLE 3.—SUPERSENSITIZATION BY PYRAZOLE TYPE COMPOUNDS  
(Addendum)

| Example No. | Dye No.,<br>80 mg. per<br>mole of<br>silver | Addendum .3<br>to 10 g./mole<br>silver | Relative<br>speed | $\gamma$ | Fog      |
|-------------|---------------------------------------------|----------------------------------------|-------------------|----------|----------|
| 40          | 1(a)                                        | A                                      | None              | 100      | 2.40 .06 |
|             | 1(b)                                        | A                                      | VII               | 170      | 2.74 .06 |
|             | 1(c)                                        | A                                      | I                 | 182      | 2.40 .08 |
| 45          | 2(a)                                        | B                                      | None              | 100      | 1.95 .06 |
|             | 2(b)                                        | B                                      | I                 | 174      | 1.99 .06 |
|             | 3(a)                                        | A                                      | None              | 100      | 2.34 .06 |
|             | 3(b)                                        | A                                      | II                | 234      | 2.72 .08 |
|             | 3(c)                                        | A                                      | V                 | 112      | 2.78 .06 |
|             | 3(d)                                        | A                                      | VI                | 214      | 2.70 .08 |
|             | 3(e)                                        | A                                      | III               | 200      | 2.70 .08 |
| 50          | 4(a)                                        | B                                      | None              | 100      | 2.06 .06 |
|             | 4(b)                                        | B                                      | IV                | 155      | 1.96 .09 |
|             | 4(c)                                        | B                                      | II                | 151      | 1.90 .06 |
|             | 4(d)                                        | B                                      | VI                | 151      | 2.04 .06 |
|             | 4(e)                                        | B                                      | III               | 123      | 2.02 .06 |
|             | 4(f)                                        | B                                      | VII               | 347      | 2.02 .08 |
|             | 5(a)                                        | G                                      | None              | 100      | 2.54 .06 |
|             | 5(b)                                        | G                                      | IV                | 120      | 2.48 .08 |
|             | 5(c)                                        | G                                      | VII               | 118      | 2.78 .06 |
|             | 6(a)                                        | H                                      | None              | 100      | 2.46 .06 |
|             | 6(b)                                        | H                                      | IV                | 186      | 2.40 .08 |
|             | 6(c)                                        | H                                      | II                | 269      | 2.32 .12 |
| 55          | 6(d)                                        | H                                      | VII               | 263      | 2.38 .06 |
|             | 7(a)                                        | K                                      | None              | 100      | 2.60 .07 |
|             | 7(b)                                        | K                                      | IV                | 141      | 2.72 .07 |
|             | 7(c)                                        | K                                      | II                | 148      | 2.74 .08 |
|             | 7(d)                                        | K                                      | VII               | 155      | 2.90 .08 |
|             | 8(a)                                        | E                                      | None              | 100      | 2.46 .06 |
|             | 8(b)                                        | E                                      | IV                | 214      | 2.28 .08 |
|             | 8(c)                                        | E                                      | II                | 229      | 2.22 .06 |
| 60          | 8(d)                                        | E                                      | VII               | 339      | 2.30 .06 |
|             | 9(a)                                        | C                                      | None              | 100      | 1.98 .06 |
|             | 9(b)                                        | C                                      | VII               | 355      | 2.50 .07 |
|             | 10(a)                                       | J                                      | None              | 100      | 2.46 .08 |
|             | 10(b)                                       | J                                      | VII               | 151      | 2.44 .08 |
|             | 11(a)                                       | F                                      | None              | 100      | 2.38 .09 |
|             | 11(b)                                       | F                                      | VII               | 692      | 1.58 .11 |
| 65          | 12(a)                                       | I                                      | None              | 100      | 2.52 .08 |
|             | 12(b)                                       | I                                      | VII               | 309      | 2.28 .12 |
|             | 13(a)                                       | D                                      | None              | 100      | 3.10 .08 |
|             | 13(b)                                       | D                                      | VII               | 204      | 2.64 .08 |
|             | 14(a)                                       | A                                      | None              | 100      | 2.62 .08 |
|             | 14(b)                                       | A                                      | IX                | 132      | 2.20 .07 |
|             | 14(c)                                       | A                                      | X                 | 214      | 2.30 .48 |
|             | 15(a)                                       | A                                      | None              | 100      | 2.96 .07 |
| 70          | 15(b)                                       | A                                      | VIII              | 138      | 2.45 .06 |
|             | 16(a)                                       | Z                                      | None              | 100      | 1.28 .05 |
|             | 16(b)                                       | Z                                      | XI                | 191      | 1.43 .04 |
|             | 17(a)                                       | A                                      | None              | 100      | 1.08 .05 |
|             | 17(b)                                       | A                                      | XI                | 151      | 0.84 .04 |
|             | 18(a)                                       | Y                                      | None              | 100      | 1.62 .04 |
|             | 18(b)                                       | Y                                      | XII               | 407      | 0.96 .06 |

Referring to above Table 3, it will be seen that the relative speeds for each of the supersensitizing combinations is markedly greater than that of the control which contains the specified dye but contains no supersensitizing addendum.

The following Table 4 is included here to show the results from a concentration series wherein Dye No. A is kept constant at a concentration of 80 mg./mole of silver while Compound No. I is varied over the range of from 0.0 to 3.0 g./mole of silver.

TABLE 4

| Example No. | Concentration compound<br>No. I (g./mole<br>silver) | Relative<br>speed | $\gamma$ | Fog |
|-------------|-----------------------------------------------------|-------------------|----------|-----|
| 19(a)-----  | 0.0                                                 | 100               | 2.74     | .06 |
| 19(b)-----  | 0.03                                                | 138               | 2.34     | .08 |
| 19(c)-----  | 0.3                                                 | 191               | 2.30     | .08 |
| 19(d)-----  | 3.0                                                 | 110               | 2.82     | .08 |
| 19(e)-----  | 1.0                                                 | 182               | 2.02     | .07 |

These data indicate that the optimum concentration of the addendum in the supersensitizing combinations of the invention are as previously mentioned generally in the range of about 0.3 to 1.0 g./mole of silver.

## EXAMPLES 20 TO 44

These examples illustrate the supersensitization produced with the tetrazoles and tetrazolium salts in combination with various methine dyes coming under the definitions of Formulas IV to VI above. The testing procedure is exactly the same as that described in the preceding examples and the results are tabulated in similar manner in the following Table 5.

TABLE 5.—SUPERSENSITIZATION BY TETRAZOLE TYPE COMPOUNDS [Addendum]

| Example No. | Dye No. and conc. (g./mole silver) | Addendum and conc. supersensi-<br>tizer (g./mole silver) | Relative speed | $\gamma$ | Fog |
|-------------|------------------------------------|----------------------------------------------------------|----------------|----------|-----|
| 20(a)-----  | A (0.053)                          | None-----                                                | 100            | 3.22     | .07 |
| 20(b)-----  | A (0.053)                          | XX (0.75)-----                                           | 115            | 3.06     | .06 |
| 21(a)-----  | P (0.05)                           | None-----                                                | 100            | 2.80     | .08 |
| 21(b)-----  | P (0.05)                           | XXII (0.3)-----                                          | 436            | 3.90     | .33 |
| 22(a)-----  | P (0.08)                           | None-----                                                | 100            | 3.90     | .07 |
| 22(b)-----  | P (0.08)                           | XX (3.0)-----                                            | 269            | 5.40     | .06 |
| 23(a)-----  | P (0.030)                          | None-----                                                | 100            | 2.82     | .08 |
| 23(b)-----  | P (0.030)                          | XV (3.0)-----                                            | 251            | 4.15     | .07 |
| 23(c)-----  | P (0.030)                          | XIX (3.0)-----                                           | 148            | 3.80     | .07 |
| 23(d)-----  | P (0.030)                          | XXVI (3.0)-----                                          | 355            | 3.64     | .07 |
| 24(a)-----  | D (0.03)                           | None-----                                                | 100            | 3.28     | .07 |
| 24(b)-----  | D (0.03)                           | XX (3.0)-----                                            | 380            | 3.24     | .06 |
| 24(c)-----  | D (0.03)                           | XXII (0.3)-----                                          | 427            | 4.40     | .05 |
| 25(a)-----  | T (0.04)                           | None-----                                                | 100            | 3.44     | .06 |
| 25(b)-----  | T (0.04)                           | XX (3.0)-----                                            | 191            | 3.12     | .05 |
| 26(a)-----  | S (0.015)                          | None-----                                                | 100            | 2.80     | .06 |
| 26(b)-----  | S (0.015)                          | XX (3.0)-----                                            | 257            | 3.20     | .05 |
| 26(c)-----  | S (0.015)                          | XXII (0.3)-----                                          | 240            | 4.60     | .06 |
| 27(a)-----  | U (0.015)                          | None-----                                                | 100            | 3.04     | .08 |
| 27(b)-----  | U (0.015)                          | XX (3.0)-----                                            | 129            | 3.60     | .06 |
| 28(a)-----  | R (0.015)                          | None-----                                                | 100            | 3.04     | .08 |
| 28(b)-----  | R (0.015)                          | XX (3.0)-----                                            | 186            | 2.74     | .07 |
| 29(a)-----  | A (0.06)                           | None-----                                                | 100            | 2.90     | .07 |
| 29(b)-----  | A (0.06)                           | XIV-----                                                 | 138            | 2.80     | .07 |
| 30(a)-----  | L (0.08)                           | None-----                                                | 100            | 1.30     | .06 |
| 30(b)-----  | L (0.08)                           | XXII (0.3)-----                                          | 209            | 3.40     | .06 |
| 31(a)-----  | M (0.08)                           | None-----                                                | 100            | 1.30     | .07 |
| 31(b)-----  | M (0.08)                           | XXII (0.3)-----                                          | 178            | 3.10     | .07 |
| 32(a)-----  | B (0.05)                           | None-----                                                | 100            | 1.60     | .07 |
| 32(b)-----  | B (0.05)                           | XXII (0.3)-----                                          | 631            | 3.16     | .06 |
| 33(a)-----  | Q (0.033)                          | None-----                                                | 100            | 2.50     | .05 |
| 33(b)-----  | Q (0.033)                          | XXII (0.3)-----                                          | 289            | 3.26     | .06 |
| 34(a)-----  | X (0.04)                           | None-----                                                | 100            | -----    | .08 |
| 34(b)-----  | X (0.04)                           | XXII (0.3)-----                                          | 1,200          | 3.28     | .13 |
| 35(a)-----  | A (0.05)                           | None-----                                                | 100            | 2.75     | .08 |
| 35(b)-----  | A (0.05)                           | XX (3.0)-----                                            | 141            | 2.84     | .03 |
| 35(c)-----  | A (0.05)                           | XXII (3.0)-----                                          | 151            | 2.68     | .07 |
| 36(a)-----  | C (0.115)                          | None-----                                                | 100            | 2.16     | .06 |
| 36(b)-----  | C (0.115)                          | XX (3.0)-----                                            | 282            | 2.98     | .06 |
| 36(c)-----  | C (0.115)                          | XV (3.0)-----                                            | 162            | 2.80     | .05 |
| 37(a)-----  | B (0.080)                          | None-----                                                | 100            | 2.14     | .07 |
| 37(b)-----  | B (0.080)                          | XX (3.0)-----                                            | 141            | 3.00     | .04 |
| 37(c)-----  | B (0.080)                          | XV (3.0)-----                                            | 151            | 2.64     | .65 |
| (38a)-----  | O (0.115)                          | None-----                                                | 100            | 2.57     | .06 |

TABLE 5.—Continued

| 5            | Example No. | Dye No. and conc. (g./mole silver) | Addendum and conc. supersensi-<br>tizer (g./mole silver) | Relative speed | $\gamma$ | Fog |
|--------------|-------------|------------------------------------|----------------------------------------------------------|----------------|----------|-----|
| 38(b)-----   | O (0.115)   | XII (1.5)-----                     | 178                                                      | 2.44           | .04      |     |
| 38(c)-----   | O (0.115)   | XV (3.0)-----                      | 309                                                      | 3.18           | .03      |     |
| 38(d)-----   | O (0.115)   | XVII (3.0)-----                    | 513                                                      | 3.26           | .03      |     |
| 38(e)-----   | O (0.115)   | XX (3.0)-----                      | 417                                                      | 3.30           | .03      |     |
| 38(f)-----   | O (0.115)   | XXV (0.3)-----                     | 166                                                      | 2.36           | .03      |     |
| 38(g)-----   | O (0.115)   | XXI (1.5)-----                     | 219                                                      | 2.22           | .04      |     |
| 39(a)-----   | V (0.115)   | None-----                          | 100                                                      | 3.18           | .04      |     |
| 39(b)-----   | V (0.115)   | XX (3.0)-----                      | 155                                                      | 3.14           | .03      |     |
| 40 (a)-----  | W (0.115)   | None-----                          | 100                                                      | 1.70           | .04      |     |
| 40 (b)-----  | W (0.115)   | XIII (1.5)-----                    | 110                                                      | 2.30           | .04      |     |
| 40 (c)-----  | W (0.115)   | XV (3.0)-----                      | 132                                                      | 3.18           | .03      |     |
| 41 (a)-----  | V (0.1)     | None-----                          | 100                                                      | 2.40           | .03      |     |
| 41 (b)-----  | V (0.1)     | XXIII (3.0)-----                   | 398                                                      | 2.70           | .03      |     |
| 42 (a)-----  | C (0.12)    | None-----                          | 100                                                      | 1.47           | .03      |     |
| 42 (b)-----  | C (0.12)    | XXIII (3.0)-----                   | 501                                                      | 2.04           | .03      |     |
| 43 (a)-----  | B (0.1)     | None-----                          | 100                                                      | 1.80           | .03      |     |
| 43 (b)-----  | B (0.1)     | XXIII (3.0)-----                   | 468                                                      | 2.00           | .03      |     |
| 44 (a)-----  | C (0.12)    | None-----                          | 100                                                      | 1.74           | .04      |     |
| 44 (b)-----  | C (0.12)    | XXIV (3.0)-----                    | 347                                                      | 2.76           | .03      |     |
| 44A (a)----- | Y (0.076)   | None-----                          | 100                                                      | -----          | -----    |     |
| 44A (b)----- | Y (0.076)   | XXVIA-----                         | 290                                                      | -----          | -----    |     |

It will be noted from above Table 5 that in each instance substantial improvement in relative speed over each dye alone is shown by the supersensitizing combinations of the invention.

## EXAMPLES 45-57

These examples illustrate the supersensitization produced with the triazoles and imidazole compounds of the invention in combination with various methine dyes coming under the definitions of Formulas IV to VI above. The testing procedure is exactly the same as that described in the preceding examples and the results are tabulated in similar manner in the following Table 6.

TABLE 6.—SUPERSENSITIZATION BY TRIAZOLE AND IMIDAZOLE TYPE COMPOUNDS [Addendum]

| 40          | Example No. | Dye No. and conc. (g./mole silver) | Addendum and conc. (g./mole silver) | Relative speed | $\gamma$ | Fog |
|-------------|-------------|------------------------------------|-------------------------------------|----------------|----------|-----|
| 45 (a)----- | Y (0.076)   | None-----                          | 100                                 | 1.32           | .06      |     |
| 45 (b)----- | Y (0.076)   | XXVII (0.33)-----                  | 6,170                               | 1.40           | .06      |     |
| 46 (a)----- | Y (0.076)   | None-----                          | 100                                 | 1.50           | .06      |     |
| 46 (b)----- | Y (0.076)   | XXVIII (1.0)-----                  | 6,460                               | 1.68           | .06      |     |
| 46 (c)----- | Y (0.076)   | XXIX (0.66)-----                   | 75,900                              | 1.33           | .05      |     |
| 47 (a)----- | Z (0.066)   | None-----                          | 100                                 | 1.28           | .05      |     |
| 47 (b)----- | Z (0.066)   | XXXVI (0.3)-----                   | 191                                 | 1.18           | .12      |     |
| 48 (a)----- | D (0.053)   | None-----                          | 100                                 | 0.96           | .04      |     |
| 48 (b)----- | D (0.053)   | XXXVII (0.6)-----                  | 436                                 | 1.16           | .06      |     |
| 49 (a)----- | P' (0.05)   | None-----                          | 100                                 | 1.36           | .04      |     |
| 49 (b)----- | P' (0.05)   | XXX (0.66)-----                    | 115                                 | 1.24           | .04      |     |
| 50 (a)----- | I (0.04)    | None-----                          | 100                                 | 1.34           | .05      |     |
| 50 (b)----- | I (0.04)    | XXXIV (0.33)-----                  | 162                                 | 1.15           | .05      |     |
| 50 (c)----- | I (0.04)    | XXXVI (0.3)-----                   | 138                                 | 1.02           | .14      |     |
| 50 (d)----- | I (0.04)    | XXV (3.0)-----                     | 186                                 | 0.79           | .05      |     |
| 50 (e)----- | I (0.04)    | XXXVII (0.6)-----                  | 178                                 | 1.10           | .05      |     |
| 51 (a)----- | Y (0.076)   | None-----                          | 100                                 | 1.70           | .06      |     |
| 51 (b)----- | Y (0.076)   | XXXV (3.0)-----                    | 5,750                               | 1.59           | .06      |     |
| 51 (c)----- | Y (0.076)   | XXXVII (0.6)-----                  | 55,000                              | 1.50           | .05      |     |
| 52 (a)----- | W (0.076)   | None-----                          | 100                                 | 1.55           | .04      |     |
| 52 (b)----- | W (0.076)   | XXXVII (0.6)-----                  | 132                                 | 1.40           | .05      |     |
| 53 (a)----- | A (0.066)   | None-----                          | 100                                 | 1.08           | .05      |     |
| 53 (b)----- | A (0.066)   | XXXVI (0.3)-----                   | 151                                 | 0.88           | .23      |     |
| 54 (a)----- | Y (0.076)   | None-----                          | 100                                 | 0.96           | .04      |     |
| 54 (b)----- | Y (0.076)   | XXXIII (0.1)-----                  | 1,380                               | 1.48           | .04      |     |
| 54 (c)----- | Y (0.076)   | XXXII (0.3)-----                   | 759                                 | 1.18           | .04      |     |
| 54 (d)----- | Y (0.076)   | XXXI (0.3)-----                    | 631                                 | 1.74           | .04      |     |
| 55 (a)----- | Y (0.076)   | None-----                          | 100                                 | 1.00           | .04      |     |
| 55 (b)----- | Y (0.076)   | XXXVIII (0.1)-----                 | 2,240                               | 1.18           | .04      |     |
| 55 (c)----- | Y (0.076)   | XXXIX (0.1)-----                   | 3,310                               | 1.24           | .04      |     |
| 56 (a)----- | Y (0.076)   | None-----                          | 100                                 | 0.96           | .04      |     |
| 56 (b)----- | Y (0.076)   | XL (1.0)-----                      | 871                                 | 1.32           | .04      |     |
| 57 (a)----- | Y (0.076)   | None-----                          | 100                                 | 0.63           | .04      |     |
| 57 (b)----- | Y (0.076)   | XL (1.0)-----                      | 398                                 | 1.04           | .04      |     |

Referring to above Table 6, it will be observed that the relative speed for each of the specified supersensitizing combinations is markedly greater than that of the control

## 11

example containing the dye alone, i.e., without the supersensitizing addendum. Remarkably high relative speeds are shown for Example 46 (c) comprising Dye No. Y and addendum Compound No. XXIX, and Example 51(c) comprising Dye No. Y and addendum Compound No. XXXVII, with no increase in fog in each instance.

It will be apparent from all of the foregoing description that still other combinations of the invention can be produced by appropriate selection of other heterocyclic compounds of the type described herein with other photographic methine dyes and that such combinations likewise will result in supersensitized photographic silver halide emulsions.

The invention has been described in detail with particular reference to preferred embodiments thereof, but, it will be understood that variations and modifications can be effected within the spirit and scope of the invention described hereinabove and in the appended claims.

I claim:

1. A photographic silver halide emulsion containing a supersensitizing combination of (1) a heterocyclic compound having the following formula:



wherein R<sub>9</sub> and R<sub>11</sub> each represents a member selected from the group consisting of a hydrogen atom or an aryl group; and, R<sub>10</sub> represents a member selected from the group consisting of hydrogen and amino; and (2) a photographic spectral sensitizing methine dye selected from those having one of the following formulas:



and



wherein n and e each represents a positive integer of from 1 to 2; d and m each represents a positive integer of from 1 to 3; R<sub>1</sub> and R<sub>2</sub> each represents a member selected from the group consisting of an alkyl group and an aryl group; X represents an acid anion; Z and Z<sub>1</sub> each represents the non-metallic atoms necessary to complete a nucleus selected from the group consisting of a thiazole nucleus, an oxazole nucleus, a selenazole nucleus, a thiazoline nucleus, a pyridine nucleus, a 3,3-dialkyl-indolenine nucleus, a quinoline nucleus and an imidazole nucleus; L repre-

## 12

sents a methine linkage; and, Q represents the non-metallic atoms necessary to complete a heterocyclic ketomethylene nucleus selected from the group consisting of a 2-pyrazolin-5-one nucleus, an isoxazolone nucleus, an oxindole nucleus, a 2,4,6-triketohexahydropyrimidine nucleus, a rhodanine nucleus, a 2(3H)-imidazo[1,2-a]pyridone nucleus, a 5,7-dioxo-6,7-dihydro-5-thiazolo[3,2-a]pyrimidine nucleus, a 2-thio-2,4-oxazolidinedione nucleus, a thianaphthenone nucleus, a 2-thio-2,5-thiazolidinedione nucleus, a 2,4-thiazolidinedione nucleus, a thiazolidinone nucleus, a 2-thiazolin-4-one nucleus, a 2-imino-4-oxazolidinone nucleus, a 2,4-imidazolidinedione nucleus, a 2-thio-2,4-imidazolidinedione nucleus, and a 2-imidazolin-5-one nucleus.

5 15 20 25 30 35 40 45 50 55 60 65 70 75 80 85 90 95 100

2. A photographic silver halide emulsion comprising a supersensitizing combination of (1) a heterocyclic compound selected from the group consisting of

3-amino-5-phenyl-1,2,4-triazole,  
3,3'-bis(1,5-diphenyl-1,2,4-triazole),  
1,5-diphenyl-1,2,4-triazole,  
4-amino-3,5-di-(p-aminophenyl)-1,2,4-triazole,  
poly(1,2,4-triazole),  
4-(5-cyanomethyl-1-phenyl-1,2,4-triazol-3-yl)benzaldehyde-N-chlorophenylhydrazone,  
3,3'-p-phenylenebis-(5-cyanomethyl-1-phenyl-1,2,4-triazole),

and (2) a methine dye selected from the group consisting of 3,3'-di-β-hydroxyethylthiadicyanine salt and 5-[di(1-ethyl-2(1H-β-naphthothiazolylidene)isopropylidene]-1,3-di(β-methoxyethyl)-barbituric acid.

3. A photographic silver halide emulsion comprising a supersensitizing combination of (1) the heterocyclic compound 1,5-diphenyl-1,2,4-triazole and (2) the methine dye 5-[di(1-ethyl-2(1H)-β-naphthothiazolylidene)isopropylidene]-1,3-di-β-methoxyethyl)-barbituric acid.

4. A photographic element comprising a support having a coating thereon containing an emulsion of claim 1.

5. A photographic element comprising a support having a coating thereon containing an emulsion of claim 2.

6. A photographic element comprising a support having a coating thereon containing an emulsion of claim 3.

## References Cited

| UNITED STATES PATENTS |         |                 |        |
|-----------------------|---------|-----------------|--------|
| 2,271,623             | 2/1942  | Carroll         | 96—104 |
| 2,566,167             | 8/1951  | Carroll et al.  | 96—104 |
| 2,680,686             | 6/1954  | Van Dormael     | 96—104 |
| 3,255,012             | 6/1966  | Glockner et al. | 96—74  |
| 3,397,987             | 8/1968  | Luckey et al.   | 96—109 |
| 3,411,915             | 11/1968 | Jones et al.    | 96—104 |
| 3,420,664             | 1/1969  | Dersch et al.   | 96—109 |
| 3,457,078             | 7/1969  | Riester         | 96—104 |
| 3,468,665             | 9/1969  | Misu et al.     | 96—74  |

J. TRAVIS BROWN, Primary Examiner

U.S. Cl. X.R.

96—109